

## UNITED STATES PATENT OFFICE

2,205,611

PERMANENT MAGNET AND PROCESS FOR  
PRODUCING THE SAMEGünther Wassermann, Frankfort-on-the-Main,  
Germany, assignor to American Lurgi Corpora-  
tion, New York, N. Y., a corporation of New  
YorkNo Drawing. Application November 26, 1938, Se-  
rial No. 242,636. In Germany November 26,  
1937

4 Claims. (Cl. 75—22)

The invention relates to permanent magnets and to a process for producing the same.

It is well known that permanent magnets may be made from various metals and metal alloys having magnetic characteristics. One type of alloy frequently used for this purpose contains iron, nickel and aluminum. Magnets formed from such alloys are generally produced by casting, since it is difficult to work the magnetic materials because of their great hardness. Such cast magnets have a coarse crystalline structure and are very brittle. Their resistance to mechanical blows, or to centrifugal force where they are used in rotating machines, is very low so that they are not practical for such purposes. Efforts have been made to produce magnets having greater mechanical resistance from such alloys by binding together powdered particles of the magnetic alloys with a binding agent having no ferro magnetic properties. Ingots of the alloys have been broken up, and the powder thus obtained pressed together in the presence of a binding agent. This binding agent, however, deleteriously affects the magnetic properties of the alloys, and renders the resulting articles of very low magnetic strength.

Effort has also been made to produce alloys by sintering. The powder is molded in a press under a high pressure and heated to a high sintering temperature. However, the magnets thus obtained also have low magnetic values as compared with the cast alloys, even though mechanically they are stronger. The value of the remanence is particularly low, and such magnets are practically useless.

The present invention relates to the production of iron-nickel-aluminum alloys having high magnetic properties and great mechanical strength by a sintering process. According to the invention, a mixture of powders of the different ingredients of the alloy is not merely pressed and subjected to a sintering temperature, but is first preheated to a lower temperature, again powdered, and then compressed and sintered. I have found that by this procedure an alloy of great strength which retains its magnetic qualities may be produced.

According to the invention, the three metals in the form of a powder are intimately mixed. The preheating is then carried out at a temperature higher than the melting point of the aluminum, but lower than that at which complete sintering of the different metals takes place. Preferably the heating is within the range of 650° C. to 900° C. The period for which the heating takes place

may be relatively short, as, for instance, from thirty minutes to one hour. The preheating is preferably carried out under non-oxidizing conditions, as for instance in a vacuum, or in an atmosphere of an inert gas or a reducing gas such as hydrogen. This preheating bakes the mixture together lightly by the melting of the aluminum. Preferably the mixture is then reconverted into powder form by regrinding. This pretreated powder is then subjected to a pressure as high as possible and then sintered at temperatures between 1200° C. and the fusing point of the mixture, preferably at 1300° C. during several hours.

The resulting product has a high mechanical strength, and at the same time has high magnetic qualities comparable to those of the cast alloys. Furthermore, there is no increase in volume during sintering as occurs when the metals have not been preheated according to the invention.

According to a preferred form of the invention, the size of the grains of the iron in the powder which is treated by this process is of importance, although this grain size is not a necessary feature of the invention. As disclosed in my copending application Serial No. 242,637 executed of even date herewith, the iron particles should be of such dimensions that at least a great majority of them will pass through a 250 screen. Preferably at least 60% of the iron present is in the condition of such fine particles, although the balance may contain particles as large as those which would pass through a 145 screen.

Within the scope of the invention, it is not necessary that all three metals be subjected to the preheating treatment. It is sufficient to preheat the aluminum and one of the other two metals, the third metal being added as a powder to the reground powder resulting from the preheating treatment.

The invention is applicable to iron-nickel-aluminum alloys of magnetic character in general, that is, to alloys composed essentially of these three ingredients. It is particularly applicable to alloys either composed substantially entirely of iron, nickel and aluminum, or to such alloys which contain small or moderate amounts of other metals, for instance of cobalt and/or titanium.

There are given hereafter some examples of methods of carrying out the invention.

## Example 1

Powdered iron, nickel and aluminum are mixed together. The mixture contains 65% of iron, 22% of nickel and 13% of aluminum. This mix-

5

10

15

20

25

30

35

40

45

50

55

ture is then heated for one-half hour at 700° C. in a hydrogen atmosphere. After the heating is completed, the product is reground.

This reground powder is subjected to a high pressure and then heated to a temperature of 1,250° C. for several hours. The resulting mass has a high mechanical strength and high magnetic properties.

*Example 2*

10 Iron powder is used 70% of which will pass through a 250 screen, and the remainder of which will pass through a 178 screen. 68% of this iron powder, 20% of nickel powder and 12% of aluminum powder are mixed and heated in a vacuum furnace for thirty minutes at 800° C. The product is removed and ground to a powder. The resulting powder is subjected to compression and sintered for several hours at a temperature of 1,300° C.

*Example 3*

25 The iron and aluminum powder of Example 2 are mixed and subjected to the preheating treatment of Example 2. After regrounding, the nickel powder is mixed with the iron-aluminum mixture, and the resulting product is sintered in the manner described for Example 2.

30 Within the scope of the invention, the nickel and aluminum powder may be preheated in the manner described in Example 3 and the iron powder added thereto after regrounding.

35 While I have described herein some embodiments of my invention I wish it to be understood that I do not intend to limit myself thereby except within the scope of the appended claims.

I claim:

1. A process of producing a permanent magnet which comprises sintering a pressed powder containing a mixture of iron, nickel and aluminum in proportions to produce a magnetic ma-

terial, at a temperature between about 1200° C. and the fusing point of the mixture, in which powder the aluminum and at least one of the other metals have previously been mixed and subjected to a heat treatment in powder form 5 at about 650° C. to 900° C. for thirty minutes to one hour, and the resulting product again powdered by grinding.

2. A process of producing permanent magnets of iron-nickel-aluminum alloys, which comprises 10 mixing and heating the metals in the form of powder at about 650° C. to 900° C. for thirty minutes to one hour, grinding the resulting product, and pressing and sintering the ground mixture between 1200° C. and the fusing point of 15 the mixture.

3. A process of producing permanent magnets of iron-nickel-aluminum alloys having magnetic characteristics, which comprises mixing the aluminum and one of the other metals in the 20 form of powder and heating the mixture at about 650° C. to 900° C. for thirty minutes to one hour, grinding the resulting product, adding the third metal in the form of a powder, and subjecting the mixture of the three metals under high pressures to a sintering temperature of between about 25 1200° C. and the fusing point of the mixture.

4. A permanent magnet formed by sintering a pressed powder, containing a mixture of iron, nickel and aluminum in proportions to produce 30 a magnetic material, at a temperature between about 1200° C. and the fusing point of the mixture, in which powder the aluminum and at least one of the other metals have previously been mixed and subjected to a heat treatment in powder form at about 650° C. to 900° C. for thirty 35 minutes to one hour, and the resulting product again powdered by grinding.

GÜNTER WASSERMANN. 40